

## UNITED STATES PATENT OFFICE

2,277,428

## DIAMOND ABRASIVE TOOL

Edgar W. Engle, Grosse Pointe Park, Mich., assignor to Carboloy Company, Inc., Detroit, Mich., a corporation of New York

No Drawing. Application May 31, 1939,  
Serial No. 276,585

2 Claims. (Cl. 51—309)

The present invention relates to diamond impregnated hard metal compositions and more particularly to an abrasive composition which consists of diamond particles embedded in a hard metal composition matrix which contains metal from the group copper and silver.

Prior to the present invention abrasive compositions have been made which consist of diamond particles embedded in a hard metal composition matrix consisting for example of tungsten carbide and cobalt. A composition of this character is disclosed in Taylor Patent 1,996,598.

Diamond particles employed in any grinding wheel or drill constitute a large portion of the cost of such articles and it is highly desirable that the diamonds be held firmly in position. While the cemented carbide matrix disclosed in the Taylor patent holds the diamonds firmly in position in drills, wheel dressers and the like, I have found that in abrasive wheels, cutting-off wheels, laps, and the like, it is possible to obtain even greater gripping action on the diamond particles if the cemented carbide matrix for the diamonds contains a relatively small quantity of metal from the group copper and silver.

In carrying out my invention, I employ as the matrix for the diamond particles a mixture of tungsten carbide and metal of the iron group such as cobalt to which a few per cent of copper, or silver, or both has been added. The cobalt content of the matrix may constitute from about 3 to about 25% by weight of the mixture of tungsten carbide and cobalt, the quantity of cobalt employed depending upon the work to be performed. A tool consisting of about 75½% of a mixture of WC and 16% Co, 5½% of metal from the group copper and silver and 19% diamond particles gives very satisfactory results.

The quantity of diamond particles employed in an abrasive tool may vary but in general the quantity employed will be the maximum quantity which the matrix will hold together securely. In cut-off wheels where considerable toughness is required the volume of diamond particles may constitute about 40% of the entire volume of the abrasive portion of the wheel but in a grinding wheel where such a high degree of toughness is not required the diamonds may comprise about 50 to 60% of the entire volume. If larger volumes of diamonds than those noted above are employed, it may be found that with diamonds within mesh limits of 20 to 120, there is not enough matrix material to grip all the diamonds.

As the percentage volume of diamonds decreases the matrix can be less tough, that is,

contain less cobalt, since there will be a greater thickness of matrix surrounding each diamond particle. With a given amount of wheel wear there will be more binder to be removed with wheels containing a lesser percentage by volume of diamond with the result that if the binder is too tough the tendency to glaze over the exposed diamond particles will be increased. In producing a thin disc cutting wheel with a volume relation of two parts matrix and one part diamond, I use an inherently tougher matrix than in the case of a surface grinding wheel with approximately equal volumes of diamond and matrix. Another factor which determines the composition of the matrix is the peripheral speed at which the wheel operates. The matrix must have sufficient strength and toughness so that the wheel will not fracture from the forces developed in rotation.

20 The quantity of copper or silver or both employed in the cemented carbide matrix may vary but if too much is employed the copper or silver will glaze the wheel and prevent cutting action. A matrix consisting of about 92% or 93% of a 25 mixture of tungsten carbide and 16% cobalt with about 7% copper or 8% silver gives very satisfactory results. The diamond particles which I employ are capable of passing through a 20 to 120 mesh or even finer screen but preferably 30 are capable of passing through a 40 to 60 mesh screen about 7½ carats being employed with the above noted matrix compositions to make a small wheel about ½ inch outside diameter by  $\frac{1}{8}$  inch thick by  $\frac{1}{4}$  inch inside diameter such as used for internal grinding.

Tests carried out with abrasive wheels  $\frac{1}{2}$  inch in diameter by  $\frac{1}{8}$  inch thick with  $\frac{1}{8}$  inch hole containing about 7½ carats of diamonds of 40 to 60 mesh embedded in a cemented carbide matrix consisting of about 93% of a mixture of tungsten carbide and 16% cobalt with 7% added cobalt gave the following results:

| 45 | Weight in grams of cemented carbide removed from test block | Wheel wear in change of diameter | Grams of test block removed per .001" reduction in wheel diameter |
|----|-------------------------------------------------------------|----------------------------------|-------------------------------------------------------------------|
| 50 | 4.976 .....                                                 | .003                             | 1.659                                                             |

Similar wheels containing the same quantity and size of diamond particles embedded in a cemented carbide matrix consisting of 91.9% of a

mixture of WC and 16% Co. with 8.1% silver gave the following results:

| Weight in grams of cemented carbide removed from test block | Wheel wear in change in diameter | Grams of test block removed per .001" reduction in wheel diameter |
|-------------------------------------------------------------|----------------------------------|-------------------------------------------------------------------|
| 5.603.....                                                  | Inches .001                      | 5.603                                                             |

Similar wheels containing the same quantity and size of diamond particles embedded in a cemented carbide matrix consisting of 93% of a mixture of tungsten carbide and 16% cobalt with 7% copper gave the following results:

| Weight in grams of cemented carbide removed from test block | Wheel wear in change of diameter | Grams of test block removed per .001" reduction in wheel diameter |
|-------------------------------------------------------------|----------------------------------|-------------------------------------------------------------------|
| 6.290.....                                                  | Inches .002                      | 3.145                                                             |

In each case the wheels were rotated at 14,000 revolutions per minute. The transverse feed was 44" per minute and the feed per cut .0005". These tests indicate clearly that the use of copper and silver, and particularly silver, as a portion of cemented carbide matrix for diamond particles produces very satisfactory results.

In the manufacture of the above abrasive tools the tungsten carbide and cobalt is thoroughly mixed for example in a ball mill. The mixed material is then spread out in a thin layer and powdered copper or silver or both added and mixed therewith, usually by hand. Thereafter the diamond particles are added. These also are hand mixed with the powdered matrix material. When mixed to the desired extent the material is placed in a mold care being taken that the diamond particles remain evenly distributed throughout the powdered metal matrix. A pressure of about 2500 to 3000 lbs. per square inch is applied to the powdered material in the mold while it has a temperature of about 1400 to 1700° C. The pressed material may be heated in any suitable atmosphere, for example in hydrogen.

What I claim as new and desire to secure by Letters Patent of the United States is:

1. An abrading tool having a portion thereof consisting of diamond particles distributed in a matrix which consists of a cemented carbide containing an appreciable quantity and up to about 8% silver.

2. An abrading tool having a portion thereof consisting of diamond particles distributed in a matrix which consists of a cemented carbide containing about 8% silver, said cemented carbide consisting of about 16% cobalt with the remainder tungsten carbide.

EDGAR W. ENGLE.